

1

2,924,874

## OXIDE COATED CATHODE SUPPORTS

Harry Huber and N'guyen Thien-Chi, Paris, France, assignors to Compagnie Generale de Telegraphie Sans Fil, a corporation of France

No Drawing. Application June 14, 1955  
Serial No. 515,527

Claims priority, application France June 18, 1954

6 Claims. (Cl. 29—182.3)

The present invention relates to cathode supports and more particularly to supports for oxide-coated cathodes.

It is known to make oxide coated cathodes by coating a nickel support, which can be of various structures, with an alkaline earth layer, for example, a layer of a mixture of barium carbonate, strontium and calcium, and by sintering the coated support at a high temperature. The nickel support used contains substances which are reducers with respect to the oxide, and the support is generally obtained by melting the nickel and reducer powders together.

The reducing agents incorporated into the nickel support usually are silicon, aluminum and magnesium or, occasionally, titanium, tantalum or tungsten in metallic form.

Cathodes obtained in this way have comparatively short life, their emissive power falling to a hundredth of its initial value, for example, after 10,000 hours operation at 850° C.

It is an object of the invention to provide a cathode having a longer useful life than the cathodes of the prior art. More particularly, the invention has for its object to provide an improved compound for the manufacture of oxide coated cathode supports. With these and other objects in view, the compound of the invention comprises nickel with an addition of from 0.1% to 10% by weight of at least one metal carbide, preferably selected from among the carbides of the following metals: W, Mo, Cr, Ta, Nb, V, Hf, Zr, Ti, La, Y, Co, Pr, Th, U, Si, Al. (The carbides of said refractory metals being particularly refractory.)

According to a preferred embodiment the compound according to the invention consists of nickel with an addition of tungsten carbide.

A compound which is particularly suitable for high output cathodes intended to be operated at high temperatures has a carbide content of from 1 to 4%, while the compound for low output cathodes operating at low temperatures will preferably have a carbide content carrying from 0.1 to 1%.

The invention will be better understood by reference to the following specification given by way of illustration only.

Nickel powder, known under the trademark "Mond," in grains of 4 to 5 $\mu$ , and powdered tungsten carbide are mixed in the proportion of 3½ gms. of carbide to 100 gms. of nickel. The carbide used may, for example, be a carbide known under the trademark "Murex" in grains of about 1 gm., having a maximum content of 6.12% by weight of carbon; no more than 0.1% of the carbon contained in said carbide is in the free state. Other specific examples by which the present invention may be realized result from the substituting for the tungsten carbide any one of the 16 other carbides of the group mentioned above.

A tablet is made up of the above composition. This tablet is sintered at the temperature of 1250° C., during

2

two hours and the cathode support is shaped according to the usual practice. A cathode is then made up by coating the support with a mixture, for instance, in molecular proportions, of 5% of calcium, 45% of strontium and 50% of barium.

Applicant has found that such a cathode still retained about 25% of its emissive power after having operated 10,000 hours.

This increase of the useful life of the cathode can be explained as follows:

It is usually considered that a requisite for a satisfactory operation of an oxide coated cathode is the permanent presence, in the alkaline-earth emissive compound forming the coating of the nickel support, of a certain proportion of barium. Now, during the operation, the barium content of the cathode gradually decreases. This loss of the barium content must be compensated as nearly as possible by the barium originating from the reduction, by the reducing agents contained in the nickel support, of the barium oxide contained in the emissive compound. This reduction takes place in the solid state by reaction on the contact surface between the compound and the support. With the metal reducers generally used, the reduction is usually fairly swift and the barium which is freed in quantities greater than necessary to offset the losses forms an intermediate level between the support and the emissive compound. These intermediate levels decrease the adherence of the emissive compound to the cathode support. This, in turn, tends to decrease the reduction of the barium oxide by the reducing agent, which makes irregular the liberation of barium.

By using, in accordance with the teaching of the invention, metal carbides as reducer, an adequate reduction rate is achieved and the above disadvantage is eliminated. On the one hand, as the carbides used are very refractory, they do not emit any vapors likely to damage the cathode. On the other hand, it is believed that the products resulting from the reaction of these carbides with the emissive compound and, more particularly, the carbide and the basic barium tungstate resulting from the reaction of tungsten carbide with this compound, react in their turn with the reducing carbide and with BaO, thus further providing free barium. This action increases the useful life of the cathode.

It is to be understood that the invention is not limited to the particular example described above. Other carbide proportions, grain sizes and carbide mixing methods could be used. Thus, for instance, it is possible to use a carbide powder having larger grains, having a size up to 30 $\mu$  and a very low carbide content, when low output cathodes, intended for operating at low temperatures, are manufactured. Further, carbide powder may be added to melted nickel in a vacuum oven.

What we claim is:

1. A cathode for electron tubes, comprising an emissive body and a support for said body, said support consisting essentially of nickel containing from 0.1 to 10% of its weight of at least one refractory metal carbide.
2. A cathode for electron tubes, comprising an emissive body and a support for said body, said support consisting essentially of nickel containing from 1 to 4% of its weight of at least one refractory metal carbide.
3. A cathode for electron tubes, comprising an emissive body and a support for said body, said support consisting essentially of nickel containing from 1 to 4% of its weight of tungsten carbide.
4. A cathode for electron tubes, comprising an emissive body and a support for said body, said support

consisting essentially of nickel containing from 0.1 to 1% of its weight of at least one refractory metal carbide.

5. A cathode for electron tubes, comprising an emissive body and a support for said body, said support consisting essentially of nickel containing from 0.1 to 1% of its weight of tungsten carbide.

6. A cathode comprising a support according to claim 1, wherein said metal carbide is selected from the group

consisting of W, Mo, Cr, Ta, Nb, V, Hf, Zr, Ti, La, Y, Co, Pr, Th, U, Si, Al.

References Cited in the file of this patent

UNITED STATES PATENTS

1,819,927 Taylor \_\_\_\_\_ Aug. 18, 1931  
2,313,227 De Bats \_\_\_\_\_ Mar. 9, 1943